

Patented Sept. 17, 1940

2,215,245

# UNITED STATES PATENT OFFICE

2,215,245

## HIGH-STRENGTH COMPRESSED FIBER PRODUCT

George D. King, Chicago, and Joseph W. Gill, Elmhurst, Ill., assignors to United States Gypsum Company, Chicago, Ill., a corporation of Illinois

No Drawing. Application July 3, 1935,  
Serial No. 29,734

13 Claims.

(Cl. 92—55)

The present invention relates to a compressed fiber product of relatively high strength and of good resistance to water and moisture.

One of the objects of the invention is to produce a compressed, rather dense fiber product which may be, in its preferential form, in the form of a board or slab which may be used as artificial lumber and which, by reason of the process used in its manufacture, is endowed with relatively great strength and good resistance to water and moisture.

A further object of the invention concerns the production of a sheet or board made from fibrated wood which has been reassembled or reconstituted into a coherent, relatively strong body by a process involving the production, from the fibers of the wood itself, of autogenously formed binders, this being effected at a temperature of between 400° and 500° F. in the absence of all extraneous sizing or binding materials; that is to say, the product consists of the reassembled woody fiber which has been made coherent by the influence of heat and applied pressure. This product is then given increased strength and resistance to moisture and water by being impregnated with a fatty-acid pitch, the pitch then being hardened within the interstices of the compressed product by means of heat.

A further object of the invention is to enhance the physical strength, and resistance to water and moisture, of a compressed wood fiber product by a process comprising the impregnation of the product with a solution comprising a fatty-acid pitch, followed by baking of the product at a temperature of from 280° to 300°, or thereabout, so as to harden the material which has been introduced into the interstices of the product and to render the same substantially insoluble in organic solvents.

Further objects of the invention will become apparent from the further description and claims hereinbelow.

The raw materials which may be employed for carrying out the present invention are lignocellulosic in character; that is to say, they are either wood or a plant material of a woody nature, although the use of cellulose itself in fairly pure form is to be construed as within the scope of the present invention. However, natural wood is by far the most desirable raw material for the purpose of carrying out the invention.

As a suitable wood, it might be mentioned that common cottonwood such as is to be found in great abundance along the lower regions of the Mississippi River, as in the States of Mississippi

and Arkansas, forms an excellent raw material. Cottonwood trees may be cut up into logs of suitable size, the bark removed, and the logs then suitably comminuted or ground. One way of accomplishing this result is to grind the logs wet, longitudinally of the fiber, using a copious amount of water to wash away the fibers as they are stripped from the wood. This process is entirely analogous to the wet grinding process employed in the manufacture of common insulating board such as has been manufactured for many years. An alternative method is to break the wood into small pieces and then to fibrate the pieces in a suitable dry-grinding mill, which will form loose fibers of wood. Any other suitable method of fibration may also be employed.

In its preferred form the invention is carried out substantially as follows:

In the production, for example, of a slab, board, or like article of artificial lumber, any suitable type of wood, such as pine, hemlock, spruce, poplar, and particularly cottonwood or the like, is fibrated by any suitable means. This may be accomplished by triturating, that is, grinding it by means of grindstones in the presence of water, or by any other means. Care is taken to avoid the removal of any of the woody material other than such parts thereof as are naturally water soluble. The fiber thus obtained is separated from the water used in the grinding by filtration by means of a centrifuge or by means of a Decker filter or other equivalent device well known in the paper industry and in the manufacture of insulating boards. The fiber thus obtained is then dried, although it is highly preferable to sheet the fiber while in water suspension by means of a board-forming machine or Fourdrinier wire into a coherent sheet.

Thus, for example, in making such a sheet the fiber may be suspended in water with a concentration of fiber in water of about 2% to 3%. Sizing material, waterproofing material or binders of any kind may be added to the fiber in the usual manner.

The suspension of fiber in water is fed to an Oliver board-forming machine, on which it is formed into a continuous mat which may vary in thickness from about  $\frac{1}{2}$  inch to  $1\frac{1}{2}$  inches. While on this machine, it is pressed between forwardly moving belts made of felt or the like, so as to express the major part of the free water, yielding a wet pulp board containing about 65% of moisture. The continuously formed damp or wet mat is automatically cut, while moving, into lengths, say, about 12 feet, and the full width of

the machine, which may vary from 8 to 24 feet, and these individual slabs or boards are then continuously transported into a hot air drier which may be of the Coe type. In this drier the boards are subjected to a continuous heated-air drying current until they have been relieved of substantially all of their moisture.

After the boards have been completely dried, and by this it should be understood that no free moisture of any kind remains in the boards—in other words, that they are bone-dry and as nearly as possible absolutely free from water in any form, they are subjected to the next step of the process, which consists in placing the boards between the platens of a hydraulic press. The platens of this press are heated, as for example by high pressure steam, so that their surface, and the surface of the caul plates that are used to protect the platens, have a temperature of not less than 400° F. and not substantially greater than 500° F. In using cottonwood, for example, a temperature between 440° and 470° F. has been found to be the most satisfactory for rapid, economical commercial operation. The boards, free from moisture, are placed between the platens of such a press, there being, say, ten platens, so that ten boards may be treated at one time. The press is then closed with comparatively light pressure, of say about 50 pounds per square inch, so that there is good contact between the heated platens or caul plates and the surface of the boards. While thus compressed, the boards will be rapidly heated, by reason of heat transferred from the heated platens or caul plates. The press preferably is kept closed for only a few minutes and is then opened, but the boards are allowed to remain in the press, this being done for the purpose of allowing the escape of any smoke or gases which may have been produced by the first incipient thermal decomposition of the woody fiber. The press is then again closed, this time a pressure within the range of 500 to 3000 pounds per square inch being applied. The pressure is allowed to remain on with full force for a few minutes, say, three or four, when it is again released for the purpose of allowing the escape of by that time rather copiously developed gases and vapors resulting from the thermolytic decomposition of the wood. What appears to be taking place is a sort of "cracking" or pyrolysis of the lignocellulosic constituents of the wood with the concomitant formation or development of resin-like or tar-like substances which will act as binders to fasten the fibers together. The intermittent release of pressure is advisable, as it permits the escape of gases and vapors which have developed and which otherwise, if their quantity became too great, would tend to blister or disrupt the board that is being made. After the release of pressure and the escape of gases and vapors, the pressure is again applied to the full extent and kept on for about the same length of time as before, whereupon it is again released and the newly formed gases and vapors permitted to escape. A third pressing may be resorted to if found necessary, but in most instances a double application of high pressure (that is, three applications of pressure all together) will usually be sufficient to produce a firmly consolidated wood board of, say, from  $\frac{1}{8}$  inch to  $\frac{1}{4}$  inch in thickness, depending upon the thickness of the dry mat which has been pressed.

The board thus made is then removed from the press and even in that form would be a commercial article of manufacture having a modulus of rupture on the order of about 5000 pounds per

square inch, or higher. In order to endow the pressed board with properties of enhanced tensile strength and resistance to water, the second part of the present process is brought into play. This is as follows:

The boards, while still hot or (if they have been allowed to cool) preferably having been reheated to a temperature of, say, 200° to 300° F., are immersed in an impregnating solution which contains a fatty-acid pitch. A suitable impregnating bath may have the following composition, viz., 300 grams of fatty-acid pitch and 700 grams of a petroleum distillate having substantially the characteristics of kerosene. To obtain additional water-resistance, a waterproofing substance, such as paraffin, may be added to the solution.

In the above formula the fatty-acid pitch is a substance that is derived from the residues remaining after the distillation of fatty acids, as for example those obtained from various oils such as cottonseed oil or from animal stearin. These fatty-acid pitches are dark brown to black substances having many of the characteristics of ordinary coal-tar pitch but with the distinction that they are capable of becoming substantially insoluble in organic solvents and become solid and substantially infusible when subjected to temperatures of from 250° to 300° F. in the presence of oxygen.

The impregnation of the hot boards with the above-mentioned pitch-containing solution is preferably effected at a temperature of from between 200° and 250° F. The time that the boards remain in the impregnating bath may vary from 20 to 30 minutes in the case of boards  $\frac{1}{8}$  inch thick to from 45 to 60 minutes in the case of boards  $\frac{1}{4}$  inch thick, and intermediate periods for boards between the stated thicknesses. During the impregnation, the boards will become substantially saturated with the fatty-acid pitch solution, so that in their finished condition the boards will contain from about 3% to 6% of pitch. After the boards have been in the impregnating bath for a sufficient length of time, they are lifted therefrom, and the excess solution is removed from the surfaces of the boards by any suitable means, as for instance by a squeegee or doctor-blade. A simple wiping may also be employed to assure that there is no excess liquid on the boards.

The impregnated boards are then placed into a tunnel or drier, preferably on edge and separated from each other so as to allow good access of air, and while in this drier are subjected to a current of heated air, preferably at a temperature of from 280° to 300° F., or higher. Care must be taken, of course, to avoid using temperatures so high as to cause possible ignition of the boards. While in this drier, the solvent—that is, the kerosene, for example—will become vaporized, and the fatty-acid pitch will be converted into a substantially infusible and insoluble substance which, deposited in the interstices of the board and on the fibers thereof, will render the board moisture and water-resistant. Furthermore, it will be found that when the process has been properly carried out the strength of the boards will be very greatly increased. For example, when working with the above preferred formula and starting with a board having a modulus of rupture of, say, 5000 to 7000 pounds per square inch, the finished impregnated and baked boards will ordinarily have a modulus of rupture of about 8000 to 11,000 pounds per square inch. The water-absorption of such a board will be on the order of about from 8% to 14%.

The fatty-acid pitches may be of any desired origin, such as cotton stearin pitch, cottonseed fatty-acid pitch, stearin pitch, or cottonseed-oil foots pitch. All of these are now available as 5 commercial products at a low cost, and for this reason the cost of carrying out the present invention is very low, so that it presents great commercial advantages.

The products obtained are a pleasing brown to 10 chocolate brown color and, because of their high modulus of rupture, lend themselves to many industrial uses. Thus, they may be employed as table tops, wall panels, packing cases, backing for signs, partitioning, paneling, and for general 15 cabinet work. Due to their high water resistance, they may also be employed in certain outside work.

A very advantageous way of carrying out the present invention is to omit all size or water- 20 proofing materials when making the original board, it having been found that the final product will thus have greater strength. When operating in the absence of size, it is helpful to use a small amount of an acid-reacting substance or 25 salt in the water in which the pulp is suspended. Such a salt may consist of aluminum sulfate, alum, copper sulfate, ferrous sulfate, ferric sulfate, nickel sulfate, or copper sulfate. The amount of such salt used may be on the order of 30 from 1% to 2% of the weight of the fibers. Hydrochloric acid and other materials may also be employed. The use of the salt or other material, however, is not absolutely essential, as it has been found that equally satisfactory products can 35 be made without it, the main advantage in the use of the same lying in the fact that in the pressing operations above described there is less sticking to the press platen than when it is omitted. This sticking may be overcome in other 40 ways.

It may be stated that the absence of all sizing materials or binders during the initial stages of the formation of the board by the conjoint use of pressure and high temperature is one of the 45 important features of the present process, for it has been conclusively demonstrated that a far better and stronger board or product is obtained in this way than if the fibers constituting the board have previously been sized or treated with 50 waterproofing agents. The strength of the un-impregnated board (expressed as modulus of rupture) may thus range from 6000 to 7000 pounds per square inch, and after impregnation and baking it may be as high as 11,000 pounds. 55 This is a totally new and unexpected result. Board made with sizing and waterproofing agents, when pressed, has a strength of about 5000 to 6000 pounds, or about 1000 pounds less than that of the unsized board.

The sized, impregnated and baked board has 60 a strength of about 7000 to 8500 pounds as compared with 10,000 to 11,000 pounds in the case of the impregnated and baked but unsized board. This is 2500 to 3000 pounds more than the sized, 65 impregnated and baked board. Thus before impregnation and baking the unsized board has about a 1000-pound advantage over the sized board, while after impregnation and baking the unsized board has an advantage of about 2500 to 70 3000 pounds over the sized board, or as much as two and one-half to three times as great.

As a third alternative, it is to be construed as 75 within the present invention to incorporate a portion of the pitch integrally with the board during its formation. Thus a pitch emulsion

may be added during the sizing operation of the fibers. The method of doing this is described in detail in the copending application of Joseph W. Gill, Serial No. 29,735, filed July 3, 1935.

The process described in said Gill application comprises the fibrillation of the ligneous material, as by grinding it up in the presence of water by means of the usual pulp stones, the resulting pulp suspension being run into a suitable tank provided with an agitator. While in said tank 10 the pulp suspension is treated with a sizing material such, for example, as rosin size in an amount approximately 1% to 2% of the weight of the fibers. There is also run into the tank up to 15 10% of a vegetable or animal fatty-acid pitch as, for example, stearin pitch, cottonseed oil fatty-acid pitch, corn oil fatty-acid pitch, or the like. Due to its viscosity and immiscibility in water, it is preferable to add the pitch in the form of an emulsion so that it will be uniformly dispersed 20 among the fibers. A solvent for the pitch is preferably added to the pitch to facilitate its emulsification. After the pitch and fibers have been mixed in the said tank, a sufficient quantity of a precipitant such as alum or aluminum sulfate is added to decompose the rosin soap size, with the formation—in the usual manner—of an 25 insoluble precipitate which deposits itself upon the fibers. The pitch that has been added to the mixture also is deposited on the fibers. The resultant suspension of treated fibers is now transferred to a suitable board-forming machine such as a Fourdrinier or Oliver board former, or other mechanically equivalent device, upon which it is formed into a wet mat. This mat is then 30 slightly compacted by being passed between squeeze rollers, all in the manner well known in this art, whereupon the resultant damp mats are transferred to a drier wherein they are dried, with the removal of all or substantially all of 35 the moisture therein contained. The pitch, by reason of the temperature used in the drier (250-350° F.), becomes somewhat hardened. It is generally desirable subsequently to store the boards for a few days, more or less, in order to 40 further increase the hardening of the pitch. 45

Instead of forming the board wet, it is possible to proceed by first producing dry fibrated wood, as by grinding the same. The thus produced fibers are then mechanically mixed with a small 50 amount of the above-mentioned pitchy substances to form fibers having these substances adhering thereto. The thus treated fibers are then stored, either hot or cold, to allow the added materials to harden somewhat. Thereupon the fibers are mechanically made into a mat, as by blowing them with an air current onto a 55 foraminous surface while applying suction to the latter.

The dry mats made by either of the above- 60 described methods are then pressed under the herein-disclosed conditions of heat and pressure, being subsequently impregnated with further quantities of pitch.

We claim:

1. The process of producing a dense compressed fiber product which comprises fibrating wood, suspending the resulting fibers in water and sheeting them into a coherent loose mat, drying the mat, compressing the same at a temperature of from 400° to 500° F. to effect bonding of the fibers by autogenously developed binders, impregnating the compressed product thus obtained with a solution containing a fatty-acid pitch, and heating the impregnated product to 70 75

expel the solvent contained in the said solution and to harden the pitch.

5 2. The process of producing a dense compressed fiber product which comprises fibrating wood, suspending the resulting fibers in water and sheeting them into a coherent loose mat, drying the mat, compressing the same at a temperature of from 440° to 460° F. to effect bonding of the fibers by autogenously developed binders, impregnating the compressed product thus obtained with a solution of fatty-acid pitch in a solvent, and heating the impregnated product to drive off the solvent and to harden the pitch.

10 3. The process of producing a dense compressed fiber product which comprises fibrating wood, suspending the resulting fibers in water and sheeting them into a coherent loose mat, drying the mat, compressing the same at a temperature of from 440° to 460° F. to effect bonding of the fibers by autogenously developed binders, impregnating the compressed product thus obtained with a fatty-acid pitch, and baking at about 300° F. the impregnated product to harden the pitch.

15 4. The process of producing a dense compressed fiber product which comprises consolidating wood fibers into a dense coherent mass at a temperature of from 400° to 500° F. to effect bonding of the fibers by autogenously developed binders, impregnating the compressed product thus obtained with a fatty-acid pitch, and heating the impregnated product to harden the pitch.

20 5. The process of producing a dense compressed fiber product which comprises consolidating wood fibers into a dense coherent mass at a temperature of from 440° to 460° F. to effect bonding of the fibers by autogenously developed binders, impregnating the compressed product thus obtained with a fatty-acid pitch, and baking the impregnated product to harden the pitch.

25 6. The process of producing artificial lumber from lignocellulosic fibers, which comprises adding a fatty-acid pitch to lignocellulosic fibers, compacting the fibers and pitch while dry at a temperature of not less than 400° F., impregnating the compacted product with a further quantity of fatty-acid pitch, and then heating the product to harden the pitch.

30 7. The process of producing artificial lumber from lignocellulosic fibers which comprises adding a waterproofing material and a small amount of a fatty-acid pitch to lignocellulosic fibers, compacting the treated fibers while dry at a temperature of at least 400° F. for a time sufficient to cause the formation of autogenous pyrolytic decomposition products, impregnating the compacted product with additional fatty-acid pitch, and then heating the product to harden the pitch.

35 8. The process of producing artificial lumber

which comprises precipitating a fatty-acid pitch and a metallic resinate upon ligneous fibers, drying the resulting mixture until completely free from moisture, compacting the same at a temperature of not less than 400° F., impregnating the compacted product with a further quantity of fatty-acid pitch, and then heating the product to harden the pitch.

5 9. The process of producing artificial lumber which comprises causing a fatty-acid pitch and a metallic resinate to adhere to ligneous fibers, producing a loosely compressed but coherent mat from the latter, drying the mat until completely free from moisture, compressing the mat at a temperature of between 400° and 500° F., impregnating the resulting compressed product with a fatty-acid pitch and baking the impregnated product.

10 10. The process of producing an artificial board which comprises suspending wood or woody fibers in a solution of an acid-reacting substance, filtering the suspension to form a coherent sheet, completely drying the latter, compressing it at a temperature between 400° F. and 500° F. to form a relatively dense board, impregnating the latter with a solution of a fatty-acid pitch in an organic solvent, driving off the solvent, and baking the board at about 300° F.

15 11. The process of producing an artificial board which comprises suspending wood or woody fibers in water only, filtering the suspension to form a coherent sheet, completely drying the latter, compressing it at a temperature between 400° F. and 500° F. to form a relatively dense board, impregnating the latter with a solution of a fatty-acid pitch in an organic solvent, driving off the solvent, and baking the board at about 300° F.

20 12. The process of producing an artificial board which comprises suspending unsized wood or woody fibers merely in water, filtering the suspension to form a coherent sheet, completely drying the latter, compressing it at a temperature between 400° F. and 500° F. to form a relatively dense board, impregnating the latter with a solution of a fatty-acid pitch in an organic solvent, driving off the solvent, and baking the board at about 300° F.

25 13. The process of producing an artificial board which comprises sizing wood or woody fibers while in suspension in water, filtering the suspension to form a coherent sheet, completely drying the latter, compressing it at a temperature between 400° F. and 500° F. to form a relatively dense board, impregnating the latter with a solution of a fatty-acid pitch in an organic solvent, driving off the solvent, and baking the board at about 300° F.

30 GEORGE D. KING.  
JOSEPH W. GILL. 60